

## UNITED STATES PATENT OFFICE

2,358,011

## TREATMENT OF HYDROCARBONS

Vladimir N. Ipatieff and Louis Schmerling, Chicago, Ill., assignors to Universal Oil Products Company, Chicago, Ill., a corporation of Delaware

No Drawing. Application October 7, 1942,  
Serial No. 461,204

23 Claims. (Cl. 260—683.4)

This is a continuation-in-part of our co-pending application Serial No. 443,008, filed May 14, 1942.

This invention relates to the treatment of hydrocarbons in the presence of a particular type of catalyst to produce branched chain hydrocarbons. The reactions to which the invention refers more particularly may involve the alkylation of isoparaffinic, naphthenic, and aromatic hydrocarbons by olefinic hydrocarbons and olefin-acting compounds; the isomerization of paraffins and naphthenes; or the polymerization of olefinic hydrocarbons.

In its broadest aspects the present invention relates to a process for producing organic compounds, particularly hydrocarbons and phenols, of branched structure by reacting convertible organic compounds in the presence of a particular type of catalyst. The production of branched hydrocarbons may involve the isomerization of less-branched into more-branched hydrocarbons, as the isomerization of n-butane into isobutane, the isomerization of more branched into less-branched hydrocarbons, as the conversion of dimethyl cyclopentane into methyl cyclohexane, the alkylation of saturated hydrocarbons, the dealkylation of cyclic hydrocarbons including naphthenic and aromatic hydrocarbons, the polymerization or mixed polymerization of olefins, etc.

In one specific embodiment, the present invention relates to a process for producing hydrocarbons of more-highly branched carbon chain structure than the charged hydrocarbon starting material which comprises contacting said hydrocarbon material under reaction conditions with a catalyst formed by interacting a phosphoric acid and a metal halide of the Friedel-Crafts type, separating from the reaction products the more-highly branched chain hydrocarbons and the unconverted hydrocarbon starting material, and recycling said unconverted material to further contact with the catalyst.

The hydrocarbons utilized as starting materials for the process of the present invention comprise paraffinic, olefinic, naphthenic, and aromatic hydrocarbons. The paraffins and olefins include both normal and branched chain isomers, while the naphthenes and aromatics comprise cyclic and alkylated cyclic hydrocarbons. The different types of hydrocarbons which may be converted

into branched and more-highly branched chain hydrocarbons according to the process of the present invention are hereinafter referred to more completely.

5 Isobutane is the isoparaffin commonly subjected to alkylation although higher molecular weight isoparaffins also react with olefinic hydrocarbons under similar or modified conditions of operation to produce branched chain paraffinic hydrocarbons of higher boiling point than the isoparaffinic hydrocarbons charged to the process. However, as the higher molecular weight isoparaffins, such as isopentane, isohexane, etc., are themselves valuable constituents of gasoline, they are consequently used less commonly than isobutane as charging stocks for the alkylation process. Normal paraffinic hydrocarbons which may be converted into isoparaffinic hydrocarbons by the present process comprise normal butane and higher-boiling paraffinic hydrocarbons of straight-chain structure. Similarly, mildly branched liquid paraffins may be isomerized into more-highly branched chain paraffinic hydrocarbons with substantially higher antiknock value than the less branched compounds charged to the process.

20 Naphthenic hydrocarbons which may be alkylated or isomerized according to the present process occur generally in admixture with paraffins and aromatics in different crude petroleums.

25 Of the different naphthenic hydrocarbons, also referred to as cycloparaffins, the cyclopentane, cyclohexane, alkyl cyclopentane and alkyl cyclohexane hydrocarbons are generally those which are isomerized or alkylated in the presence of a catalyst of the type herein described to produce naphthenic hydrocarbons of more-highly branched chain structures which are utilizable as constituents of high antiknock gasoline or for other purposes.

30 35 40 Aromatic hydrocarbons, such as benzene, toluene, other alkyl benzenes, naphthalene, alkyl naphthalenes, other poly-nuclear aromatics, etc. which are alkylated by olefinic hydrocarbons as hereinabove set forth, may be obtained from any source such as by distillation of coal, by the dehydrogenation of naphthenic hydrocarbons, by the dehydrogenation and cyclization of aliphatic hydrocarbons, etc. Alkyl aromatic hydrocarbons to which we herein refer include both mono-alkyl and poly-alkyl aromatic hydrocarbons which may

be converted into more highly alkylated aromatic hydrocarbons.

Olefinic hydrocarbons utilizable in the present process comprise mono-olefins having one double bond per molecule and poly-olefins having more than one double bond per molecule. Mono-olefins which may be polymerized or be utilized for alkylating isoparaffinic, naphthenic, or aromatic hydrocarbons in the presence of the catalyst herein described are either normally gaseous or normally liquid and include ethylene, propylene, butylenes, amylenes, and higher normally liquid olefins, the latter including various polymers of normally gaseous olefins. Cyclic olefins, such as cyclohexene, may also be utilized but generally not under the same conditions of operation as those employed with non-cyclic olefins. Other olefinic hydrocarbons utilizable in the present process include conjugated diolefins such as butadiene and isoprene and also non-conjugated diolefins and other poly-olefinic hydrocarbons containing more than 2 double bonds per molecule.

Alkylation of saturated hydrocarbons, including isoparaffinic, naphthenic and aromatic hydrocarbons may also be effected in the presence of the catalyst hereinafter described by reacting with the saturated hydrocarbons a substance capable of producing olefinic hydrocarbons under the conditions of operation chosen for the process. Such olefin-producing substances include alcohols, ethers, and esters capable of undergoing dehydration or splitting to form olefinic hydrocarbons containing at least 2 carbon atoms per molecule, which may be considered to be present in the reaction mixture even though possibly only as transient intermediate unsaturates which react further with the saturated hydrocarbons to produce desired reaction products. Olefinic hydrocarbons and the above mentioned olefin-producing substances are herein referred to as olefin-acting compounds. Alkyl halides are also olefin-acting compounds and may be considered as esters of halogen acids.

We have found that catalysts useful in promoting the formation of more-highly branched hydrocarbons from less-highly branched hydrocarbons may be made by interacting a phosphoric acid with a metal halide of the Friedel-Crafts type under such conditions that limited amounts of hydrogen halide are evolved which are generally from about 0.5 to about 2.0 molecular equivalents based upon the metal halide. It is apparent that since there are several phosphoric acids and a number of Friedel-Crafts type metal halides which may be interacted, a considerable number of alternative catalysts may be made although such catalysts will not necessarily be equivalent in their action in any particular hydrocarbon conversion reaction to produce more-branched chain hydrocarbons.

The phosphoric acids which may be employed in the manufacture of the present types of catalysts include orthophosphoric acid, pyrophosphoric acid, and metaphosphoric acid. While any of these three acids may be used in the production of the catalysts, the activity of various catalysts thus prepared will not necessarily be equivalent in any reaction in which they may be employed.

Friedel-Crafts type metal halides which are reacted with phosphoric acids to form catalysts useful in the present process include aluminum chloride, aluminum bromide, zinc chloride, zirconium chloride, ferric chloride, antimony chloride, bismuth chloride, and others. Substantially

anhydrous aluminum chloride is the Friedel-Crafts type catalyst usually used in hydrocarbon conversion reactions of the types mentioned herein because aluminum chloride is usually higher in catalytic activity under a given set of conditions than are other Friedel-Crafts type metal halides. However, disadvantages accompany its use in some instances on account of its high degree of activity. Thus, it must be handled in the substantial absence of water since it hydrolyzes readily and ultimately loses its catalytic activity when hydrolysis proceeds beyond a certain point. Aluminum chloride catalyst also has a tendency to form undesirable complexes with unsaturated and aromatic hydrocarbons. However, by reacting proportioned mixtures of an aluminum halide, such as aluminum chloride, and a phosphoric acid, in accordance with the present invention, catalysts of modified activities are obtained which may be utilized for promoting the formation of more-highly branched chain hydrocarbons as herein set forth.

Catalytic materials formed by the interaction of orthophosphoric acid and aluminum chloride are typical of those utilizable for promoting the process of the present invention. For example, in forming such a catalyst, equimolecular proportions of orthophosphoric acid and finely divided substantially anhydrous aluminum chloride may be mixed and interaction of these materials may be brought about by heating the mixture to a temperature of about 80° C. at which point a vigorous evolution of hydrogen chloride takes place and a pale yellowish powder-like composite results with a composition corresponding approximately to that of a compound having the formula  $\text{Cl}_2\text{AlPO}(\text{OH})_2$  in admixture with unreacted aluminum chloride. This composite has definite activity as catalyst for the isomerization and alkylation of saturated hydrocarbons.

When a mixture of phosphoric acid and aluminum chloride is heated, hydrogen chloride is evolved as hereinabove set forth and a solid catalytic material is produced, the activity of which depends upon the original proportions of phosphoric acid and aluminum chloride and also upon the amount of hydrogen chloride expelled during the mixing and heating. Active solid catalysts are formed when about 0.5 molecular proportion of hydrogen chloride is evolved per molecular proportion of aluminum chloride originally mixed with phosphoric acid. Active catalysts are also formed when even less hydrogen chloride is evolved but such catalysts are generally not solid and therefore are less suitable for use as reactor filling materials. In general, the preferred catalyst is formed by mixing equal proportions of phosphoric acid and aluminum chloride and thereafter heating the mixture at about 80° C. until 1 molecular proportion of hydrogen chloride is evolved. When the mixture of phosphoric acid and aluminum chloride is heated at a temperature substantially higher than 80° C., the catalytic activity of the resultant composite decreases if more than 1 molecular proportion of hydrogen chloride is formed based upon the aluminum chloride originally mixed with an equal molecular proportion of phosphoric acid. However, a composite with substantial catalyst activity results when equal molecular proportions of phosphoric acid and aluminum chloride are mixed and heated until 2 molecular equivalents of hydrogen chloride have been expelled. When proportionally larger amounts of aluminum chloride are mixed with

phosphoric acid and thereafter heated as herein described, composites having generally higher catalytic activities may be produced which may owe their increased activities to the presence of uncombined aluminum chloride.

Composite catalytic materials analogous to those formed by combining orthophosphoric acid and aluminum chloride can be made by reacting other phosphoric acids with aluminum chloride or with other Friedel-Crafts type metal halides such as those already mentioned. The activities of these alternative catalytic materials may vary considerably from those of higher activities made from aluminum chloride or aluminum bromide and phosphoric acids to those having catalytic activities of a lower order and thus more suitable for uses requiring catalysts of relatively lower activities. Furthermore, some of these composite materials may be active as catalysts for certain hydrocarbon conversion reactions and less active for others.

The preferred catalysts which are granular solids at ordinary temperatures may be used as such or be mixed with carrying or spacing materials of a relatively inert character such as various prepared forms of alumina, various silicas, activating carbons or chars, silicate minerals, synthetic silica-alumina type composites and acid-treated kaolin group minerals, such as, for example, the acid-treated montmorillonites of commerce some of which are known as "Filtrol," "Tonsil," etc. The preferred catalytic composites may be prepared in the presence of these carriers in relatively finely divided condition so that an intimate mixture of catalyst and carrier is produced, or they may be prepared separately and used to surface prepared granules, or mixed with finely divided carriers and formed into particles by pelleting or extrusion procedures.

In contrast to aluminum halide catalysts, the catalysts of the present invention do not form substantial amounts of complexes with unsaturated and aromatic hydrocarbons and, accordingly, they may be used in continuous processes over long periods of time with relatively little contamination by such complexes so that in many instances the catalyst life is considerably longer than the life of the corresponding aluminum halide in similar types of hydrocarbon conversion reactions.

According to the process of the present invention, a naphthenic, olefinic, or paraffinic hydrocarbon, or a mixture of an olefinic hydrocarbon with a saturated hydrocarbon selected from the isoparaffinic, naphthenic, and aromatic hydrocarbons, may be reacted in the presence of the above indicated catalyst at a temperature of from about -20° to about 150° C. to produce hydrocarbons of more-highly branched chain structure and of either substantially the same or higher molecular weight than that of the hydrocarbons charged to the process. The exact temperature needed for a particular conversion reaction is generally best determined by experiments. Such treatment of a paraffinic or naphthenic hydrocarbon generally effects an isomerization to produce hydrocarbons of substantially the same molecular weight but of more-highly branched chain structure while similar treatment of olefinic hydrocarbons, and particularly gaseous olefinic hydrocarbons, results in the formation of branched chain polymers. The reaction of an olefinic hydrocarbon with an aromatic, isoparaffinic, or naphthenic hydrocarbon produces an alkylated hydrocarbon more-branched in struc-

ture than the hydrocarbon subjected to alkylation.

In isomerizing paraffinic hydrocarbons with the type of catalysts herein described, either batch or continuous operations may be employed. In a simple batch procedure proportioned amounts of a paraffinic hydrocarbon and catalyst and minor amounts of hydrogen halide may be added to a vessel capable of withstanding moderately superatmospheric pressure and the contents heated for a time adequate to cause a desired degree of conversion. In some instances, especially where normally liquid paraffin hydrocarbons are treated, undesirable decomposition reactions may be minimized by introducing hydrogen. After a period of heating the reaction vessel may be cooled, the gaseous contents discharged, and the liquid hydrocarbon layer separated from the partly spent catalyst and fractionated to recover desired isomers and insufficiently isomerized hydrocarbons, the latter suitable for returning to further treatment.

In continuous operations the granular catalyst, either alone or on carriers, may be placed in reaction chambers and preheated mixtures of hydrocarbon along with hydrogen chloride may be passed through the catalyst bed which is maintained at an optimum temperature by exterior heating. Hydrogen may also be used in such operations if it is found that greater selectivity in the production of desired compounds is obtained thereby. The products from such a treatment may be continuously fractionated to separate light gases, hydrogen chloride, isomeric products and insufficiently isomerized hydrocarbons, the hydrogen chloride and the insufficiently converted hydrocarbons being recycled to the reaction zone for further treatment while the desired isomeric fractions are recovered.

In isomerizing paraffinic and naphthenic hydrocarbons with the types of catalysts which characterize the present invention, the temperatures employed are from about -20° to about 150° C. but preferably from about 20° to 125° C. With some of the less active but possibly more selective catalysts, still higher temperatures may be found suitable. Superatmospheric pressures may also be employed, particularly when using hydrogen and in some instances, pressures as high as 100 atmospheres may be utilized. The reaction time employed in batch operations and the space velocities of the reactants passed through a bed of catalyst in continuous operations may be varied as desired depending upon the values found to be optimum for producing high yields of desired products.

Alkylations of saturated hydrocarbons, including isoparaffinic, naphthenic, and aromatic hydrocarbons by olefinic hydrocarbons and olefin-acting compounds in the presence of a composite catalyst herein described, are carried out at temperatures of from about -20° to about 150° C. and under a pressure of from substantially atmospheric to approximately 100 atmospheres. In the hydrocarbon mixture subjected to alkylation, it is preferable to have present from about 2 to about 40 molecular proportions of saturated hydrocarbon per one molecular proportion of olefinic hydrocarbon introduced thereto. In general a higher molecular proportion of saturated hydrocarbon to olefinic hydrocarbon is employed when a normally liquid olefinic hydrocarbon is utilized than when alkylating with a normally gaseous olefin because of the fact that higher molecular weight olefins, particularly those boiling

higher than pentenes, frequently undergo depolymerization prior to or simultaneously with alkylation so that 1 molecular proportion of said normally liquid olefin can thus alkylate 2 or more molecular proportions of the saturated hydrocarbon and produce a substantially saturated alkylation product. It is frequently also desirable to introduce to the reaction mixture a relatively small amount of a hydrogen halide such as hydrogen chloride or hydrogen bromide and sometimes also to have hydrogen present in the reaction mixture but generally in a quantity not greater than about 10 mole per cent based upon the total hydrocarbons present.

The alkylation of a saturated hydrocarbon by an olefinic hydrocarbon or other olefin-acting compound may be carried out using either batch or continuous operation. Thus, in batch types operation, a finely divided catalyst formed by interacting aluminum chloride and a phosphoric acid is charged to a reactor containing a saturated hydrocarbon such as an isoparaffin, and the resultant mixture is then agitated while an olefinic fraction, or a hydrocarbon fraction containing both olefins and alkylatable saturated hydrocarbons, is added thereto in order to effect the formation of higher boiling more-highly branched chain hydrocarbons of gasoline boiling range and high antiknock value. After the reaction, the hydrocarbon layer is separated from the catalyst and the former is then fractionally distilled into unconverted hydrocarbon and alkylation product. The unconverted hydrocarbon and used catalyst may then be employed in another alkylation run.

Continuous type of alkylation treatment may be carried out by introducing a mixture of alkylatable saturated hydrocarbons and an olefin to a reactor containing a fixed bed of granular catalytic material formed by interacting substantially anhydrous aluminum chloride and a phosphoric acid as herein described. The olefin charged to alkylation may thus be introduced with a saturated alkylatable hydrocarbon or it may be directed to contact with said saturated hydrocarbon at a number of points intermediate the inlet and outlet of the alkylation zone. The conditions of temperature and pressure maintained in such an alkylation zone are generally between the approximate limits hereinabove set forth, but the exact conditions employed in any particular alkylation generally vary with the molecular weights and reactivities of the saturated and olefinic hydrocarbons reacting, the composition of the catalyst, and other factors.

It is generally advantageous to dilute the olefinic hydrocarbon or olefin-acting compound with a portion of the saturated hydrocarbon and to introduce the olefin-containing mixture at a plurality of points throughout the reaction zone rather than to add the undiluted olefinic hydrocarbon directly to the catalytic alkylation zone. In this way, a relatively high ratio of saturated hydrocarbon to olefinic hydrocarbon is readily maintained throughout the entire reaction so that alkylation is thereby favored and polymerization of the olefinic hydrocarbon is kept relatively low. The recovered mixture obtained from a continuous alkylation treatment is then conducted to a separating or fractionating zone in which unconverted alkylatable saturated hydrocarbons are separated from the alkylation product and said unconverted hydrocarbons are then recycled to further treatment in the alkylation zone of the process.

The following examples are given to illustrate

the character of results obtained by the use of the present process, although the data presented are not introduced with the intention of unduly restricting the generally broad scope of the invention.

#### EXAMPLE I

A catalyst was made by heating equimolecular proportions of aluminum chloride and orthophosphoric acid to a temperature of 80° C. until hydrogen chloride was no longer evolved. A second catalyst was similarly formed by heating equimolecular proportions of aluminum chloride and pyrophosphoric acid. Each of the catalysts so produced, in the form of a pale yellow powder, was placed in a rotatable steel autoclave along with amounts of normal butane shown in Table I and the autoclave was then closed, heated, and rotated at 100° C. for a period of four hours.

TABLE I  
*Isomerization of normal butane in the presence of a catalyst made by interacting aluminum chloride and a phosphoric acid*

|    | Run No.                                  |      |      |                     |      |
|----|------------------------------------------|------|------|---------------------|------|
|    | 1                                        | 2    | 3    | 4                   | 5    |
|    | Catalyst made from AlCl <sub>3</sub> and |      |      |                     |      |
| 35 | Orthophosphoric acid                     |      |      | Pyrophosphoric acid |      |
| 35 | Temperature, °C.....                     | 100  | 100  | 100                 | 100  |
|    | Maximum pressure, atmospheres.....       | 12   | 16   | 16                  | 17   |
| 30 | Reactants, parts by weight:              |      |      |                     |      |
|    | n-Butane.....                            | 52   | 52   | 51                  | 52   |
|    | Hydrogen chloride.....                   | 0    | 2    | 0                   | 2    |
|    | Catalyst.....                            | 5    | 5    | 6                   | 6    |
| 40 | Products, parts by weight:               |      |      |                     |      |
|    | Condensed gas.....                       | 52   | 49   | 51                  | 50   |
|    | Liquid.....                              | 0    | 0    | 0                   | 0    |
|    | Catalyst.....                            | 5    | 5.5  | 6                   | 6    |
|    | Hydrogen chloride.....                   | 0    | 1.5  | 0                   | 0.5  |
|    | Loss, uncondensed gas, etc.....          | 0    | 3    | 0                   | 3    |
| 45 | Analysis of condensed gas:               |      |      |                     |      |
|    | Isobutane.....                           | 26.6 | 27.4 | 10.2                | 21.5 |
|    | n-Butane.....                            | 71.2 | 71.6 | 89.0                | 77.6 |
|    | Pentanes.....                            | 2.2  | 1.0  | 0.8                 | 0.9  |
| 50 |                                          | 3.1  | 96.4 | 0.5                 |      |

From the above data it is noted that under the reaction conditions used the best results in isomerizing normal butane were obtained with the catalyst made from aluminum chloride and orthophosphoric acid, since the production of isobutane was 26.6% by weight in Run 1 and 25.8% (assuming the loss to be normal butane) in Run 2. In these two runs, there was no change in weight of the catalyst in Run 1 and a slight increase in weight in Run 2. The fact that the catalyst did not increase appreciably in weight during use is evidence that only small amounts of organic complexes were formed by the interaction of the hydrocarbons and the catalyst. It is worth noting that there was only a very small formation of hydrocarbons heavier than butane, and accordingly substantially all of the hydrocarbons other than isobutane could be recycled.

Runs 3, 4, and 5 in which normal butane was isomerized in contact with the catalyst made by interacting aluminum chloride and pyrophosphoric acid showed somewhat lower yields, particularly in the absence of added hydrogen chloride in Runs 3 and 5. The low yield of isobutane in Run 5 was probably due to the use of too low a temperature. In these three runs the isomerizing action was selective as shown by the relatively small amounts of products higher boiling than butanes. Again, the catalyst showed no ap-

preciable weight increases indicating substantially no formation of hydrocarbon complexes.

#### EXAMPLE II

Portions of the catalysts prepared as described in Example I were contacted with normal heptane in a rotatable steel autoclave under the conditions shown in Table 2.

TABLE 2

*Isomerization of normal heptane in the presence of catalysts made by interacting aluminum chloride and a phosphoric acid*

|                                                   | Run |    |    |     | 10 | Run No. |    |
|---------------------------------------------------|-----|----|----|-----|----|---------|----|
|                                                   | 6   | 7  | 8  | 9   |    |         |    |
| Catalyst made from $\text{AlCl}_3$ and            |     |    |    |     |    |         |    |
| Orthophosphoric acid                              |     |    |    |     | 10 | 10      | 12 |
| Pyrophosphoric acid                               |     |    |    |     | 15 |         |    |
| Temperature, °C.                                  | 100 | 27 | 50 | 100 | 20 | 25      | 30 |
| Duration, hours                                   | 4   | 4  | 4  | 4   | 25 | 30      | 35 |
| Maximum pressure, atmospheres                     |     |    |    |     | 30 |         |    |
| Reactants, parts by weight:                       |     |    |    |     | 35 |         |    |
| n-Heptane                                         | 50  | 50 | 50 | 50  |    |         |    |
| Hydrogen chloride                                 | 0   | 2  | 3  | 2   |    |         |    |
| Catalyst                                          | 10  | 8  | 4  | 6   |    |         |    |
| Products, parts by weight:                        |     |    |    |     |    |         |    |
| Condensed gas                                     | 0   | 0  | 0  | 0   |    |         |    |
| Liquid                                            | 41  | 45 | 50 | 47  |    |         |    |
| Catalyst                                          | 13  | 11 | 5  | 6   |    |         |    |
| Hydrogen chloride                                 | 0   | 1  | 0  | 0   |    |         |    |
| Loss, uncondensed gas, etc.                       | 6   | 4  | 1  | 5   |    |         |    |
| Distillation of liquid products, volume per cent: |     |    |    |     |    |         |    |
| C <sub>4</sub> and lighter paraffins              |     | 10 | 0  |     |    |         |    |
| C <sub>5</sub> and C <sub>6</sub> paraffins       | 5   | 26 | 0  | 0   |    |         |    |
| i-Heptanes                                        | 20  | 16 | 10 | 8   |    |         |    |
| n-Heptane                                         | 55  | 23 | 80 | 86  |    |         |    |
| C <sub>8</sub> and higher hydrocarbons            | 2   | 21 | 3  | 4   |    |         |    |

In run 6 on n-heptane, a higher yield of isoheptane (branched chain heptanes) was obtained at 100° C. in the absence of added hydrogen chloride than was obtained in run 7 at 27° C. in the presence of 2 parts by weight of hydrogen chloride. However, the reaction was obviously more selective in run 6 since there was less formation of products boiling above and below the heptanes and a considerably larger amount of unconverted normal heptane which could be recycled for further treatment.

In runs 8 and 9, the catalysts, made by interacting aluminum chloride and pyrophosphoric acid, showed a high degree of selectivity in that there was only small production of hydrocarbons boiling lower than isoheptanes and a large amount of normal heptane was recovered which could be recycled to further isomerizing treatment.

#### EXAMPLE III

40 parts by weight of aluminum chloride were added with stirring to 29 parts by weight of 100% phosphoric acid. The temperature of the well-stirred mixture rose from 20° to 70° C., the mixture first became putty-like in appearance and then yielded 59 parts by weight of yellow powder. This final weight corresponded to a loss of approximately 1 molecular equivalent of hydrogen chloride. On further heating at 85° C., more hydrogen chloride was evolved and 58.6 parts by weight of finely divided yellow powder was produced.

Alkylation of isobutane was then carried out by introducing 40 parts by weight of propylene during a period of 4 hours to an autoclave containing a stirred mixture of 168 parts by weight of isobutane, 25 parts by weight of the catalyst composite, and 5 parts by weight of hydrogen

chloride. During the addition of the propylene, the autoclave and contents were maintained at a constant reaction temperature. Three alkylation runs thus made at temperature of 35°, 60°, and 74° C. gave the results shown in Table 3.

TABLE 3

*Alkylation of isobutane with propylene*

|                                                 | Run No. |     |     |
|-------------------------------------------------|---------|-----|-----|
|                                                 | 10      | 11  | 12  |
| Temperature, °C.                                | 35      | 60  | 74  |
| Pressure, lbs./sq. in.                          | 145     | 198 | 93  |
| Products, per cent by wt. of propylene charged: |         |     |     |
| Propane                                         | 70      | 40  | 60  |
| Pentane-hexane fraction                         | 145     | 108 | 112 |
| Heptane fraction                                | 16      | 18  | 16  |
| Octane fraction                                 | 24      | 20  | 21  |
| Total liquid hydrocarbons                       | 205     | 206 | 195 |

The results given above show that good yields of alkylate were obtained by reacting isobutane with propylene at temperatures of between about 35° and 74° C. in the presence of the composite catalyst prepared from aluminum chloride and orthophosphoric acid. The amount of alkylation product boiling in the range of pentanes and hexanes was relatively high while octanes were present in larger amount than the heptanes. The relatively high proportion of propane formed indicated that some of the liquid product, possibly that boiling in the octane range, was produced by hydrogen transfer reaction in which propylene reacted with isobutane to produce propane and isobutylene, the latter being then utilized in alkylating isobutane to iso-octane.

#### EXAMPLE IV

53 parts by weight of powdered aluminum chloride were added with stirring to 71 parts by weight of pyro-phosphoric acid at 80° C. The resultant mixture which at first was paste-like in consistency soon had the appearance of putty and then hydrogen chloride was evolved while the mixture increased in volume due to foaming and finally yielded a porous cream-colored solid which was easily crushed to a powder. The yield of this powder indicated the loss of about 0.55 molecular proportion of hydrogen chloride per 0.4 molecular proportion of aluminum chloride and 0.4 molecular proportion of pyro-phosphoric acid so composited.

8 parts by weight of the catalyst powder so prepared, 81 parts by weight of isobutane and 20 parts by weight of propylene were charged to a rotatable steel autoclave and rotated therein at 60° C. for 4 hours under a maximum pressure of 12 atmospheres. After the reaction, the autoclave was cooled to room temperature, the products were removed therefrom and separated into 68 parts by weight of normally gaseous hydrocarbons (mainly isobutane), 22 parts by weight of liquid hydrocarbons, and 18 parts by weight of used catalyst consisting of yellow granules wetted with hydrocarbons. The used catalyst thus had admixed therewith about 10 parts by weight of normally liquid alkylation product. Fractional distillation of the liquid hydrocarbon product separated this material into 15% by volume of isobutane, 3% of hydrocarbons boiling below 75° C., 12% of a fraction boiling between 75° C. and 95° C. corresponding to heptanes, 10% of a fraction boiling between 95° and 125° C. consisting largely of octanes, 8% boiling between 125° and

150° C., 7% boiling between 150° and 200° C., and 42% boiling above 200° C.

EXAMPLE V

The preparation of the catalyst was similar to that shown in Example IV with the exception that the pyrophosphoric acid was initially at room temperature and no attention was paid to the temperature developed by addition thereto of the aluminum chloride.

An autoclave was then charged with 81 parts by weight of isobutane, 4 parts by weight of the catalyst powder, and 3 parts by weight of hydrogen chloride, after which ethylene was introduced until the pressure in the autoclave reached 30 atmospheres. The autoclave so charged was then rotated and heated at 60° C. for 4 hours during which the pressure decreased slightly, and later reached 20 atmospheres after the autoclave had cooled to room temperature. The resultant reaction mixture yielded 16 parts by weight of liquid hydrocarbons containing 19% by volume of dissolved isobutane, 31% of pentanes and hexanes boiling below 75° C., 10% of a heptane fraction boiling between 75° and 95° C., 16% of an octane fraction boiling between 95° and 125° C., 8% of a fraction boiling between 125° and 150° C. and 11% of higher boiling material.

EXAMPLE VI

Alkylation of benzene was carried out by gradually introducing 21 parts by weight of propylene during a period of 4 hours to an autoclave maintained at 25° C. and containing a stirred mixture of 80 parts by weight of benzene and 5 parts by weight of the catalyst composite described in Example III. After this treatment, the reaction mixture was removed from the autoclave, separated from the used catalyst, and fractionally distilled into 57% by volume of unconverted benzene, 25% of mono-isopropyl benzene, and 18% of higher boiling alkylated benzenes.

The novelty and utility of the process of the present invention are evident from the preceding specification and examples, although neither section is intended to unduly limit its generally broad scope.

We claim as our invention:

1. A process for producing organic compounds of branched carbon structure which comprises contacting a reactive organic compound under conversion conditions with a catalyst comprising the reaction product formed by interacting a phosphoric acid and a metal halide of the Friedel-Crafts type and liberating hydrogen halide in an amount not in excess of 2 mols for each mol of metal halide present, whereby said reaction product contains at least one halogen atom per mol.

2. A process for producing hydrocarbons of branched carbon structure which comprises contacting a hydrocarbon material under reaction conditions with a catalyst comprising the reaction product formed by interacting a phosphoric acid and a metal halide of the Friedel-Crafts type and liberating hydrogen halide in an amount not in excess of 2 mols for each mol of metal halide present, whereby said reaction product contains at least one halogen atom per mol.

3. A process for producing hydrocarbons of more-highly branched structure than that of a hydrocarbon starting material which comprises reacting said hydrocarbon material at a temperature of from about -20° to about 150° C. in

the presence of a catalyst comprising the reaction product formed by interacting a phosphoric acid and a metal halide of the Friedel-Crafts type and liberating hydrogen halide in an amount not in excess of 2 mols for each mol of metal halide present, whereby said reaction product contains at least one halogen atom per mol.

4. A process for producing substantially saturated hydrocarbons of more-highly branched structure than that of a hydrocarbon starting material which comprises reacting said hydrocarbon material at a temperature of from about -20° to about 150° C. in the presence of a catalyst formed by interacting a phosphoric acid and a metal halide of the Friedel-Crafts type.

5. A process for producing substantially saturated hydrocarbons of more-highly branched structure than that of a substantially saturated hydrocarbon starting material which comprises reacting said hydrocarbon material at a temperature of from about -20° to about 150° C. in the presence of a catalyst formed by interacting a phosphoric acid and a metal halide of the Friedel-Crafts type.

6. A process for producing substantially saturated hydrocarbons of more-highly branched structure than that of a substantially saturated hydrocarbon starting material which comprises reacting said hydrocarbon material and an olefinic hydrocarbon at a temperature of from about -20° to about 150° C. in the presence of a catalyst formed by interacting a phosphoric acid and a metal halide of the Friedel-Crafts type.

7. A process for producing hydrocarbons of more-highly branched structure than that of a hydrocarbon starting material which comprises reacting said hydrocarbon material at a temperature of from about -20° to about 150° C. in the presence of a catalyst comprising the reaction product formed by mixing a phosphoric acid and a tri-valent metal halide of the Friedel-Crafts type and heating the resultant mixture to cause interaction of the acid and metal halide so as to evolve from about 0.5 to about 2.0 molecular proportions of hydrogen halide per molecular proportion of metal halide interacted with said phosphoric acid, whereby said reaction product contains at least one halogen atom per mol.

8. A process for producing substantially saturated hydrocarbons of more-highly branched structure than that of a substantially saturated hydrocarbon starting material which comprises reacting said hydrocarbon material at a temperature of from about -20° to about 150° C. in the presence of a catalyst formed by interacting a phosphoric acid and a metal halide of the Friedel-Crafts type and heating the resultant mixture to cause interaction of the acid and metal halide so as to evolve from about 0.5 to about 2.0 molecular proportions of hydrogen halide per molecular proportion of metal halide interacted with said phosphoric acid.

9. A process for producing substantially saturated hydrocarbons of more-highly branched structure than that of a substantially saturated hydrocarbon starting material which comprises reacting said hydrocarbon material and an olefinic hydrocarbon at a temperature of from about -20° to about 150° C. in the presence of a catalyst formed by interacting a phosphoric acid and a metal halide of the Friedel-Crafts type and heating the resultant mixture to cause interaction of the acid and metal halide so as to evolve from about 0.5 to about 2.0 molecular proportions of hydrogen halide per molecular proportion of

metal halide interacted with said phosphoric acid.

10. The process of claim 8 further characterized in that said metal halide comprises substantially anhydrous aluminum chloride.

11. The process of claim 8 further characterized in that said phosphoric acid comprises orthophosphoric acid.

12. The process of claim 8 further characterized in that said substantially saturated hydrocarbon starting material comprises a paraffinic hydrocarbon isomerizable to a more-highly branched paraffinic hydrocarbon.

13. An alkylation process which comprises reacting an alkylatable hydrocarbon with an olefinic hydrocarbon at a temperature of from about -20° to about 150° C. in the presence of a catalyst formed by interacting a phosphoric acid and aluminum chloride and heating the resultant mixture to cause interaction of the acid and aluminum chloride to as to evolve from about 0.5 to about 2.0 molecular proportions of hydrogen chloride per molecular proportion of aluminum chloride interacted with said phosphoric acid.

14. The process of claim 13 further characterized in that said alkylatable hydrocarbon comprises an isoparaffinic hydrocarbon.

15. The process of claim 13 further characterized in that said alkylatable hydrocarbon comprises an alkylatable naphthenic hydrocarbon.

16. The process of claim 13 further characterized in that said alkylatable hydrocarbon comprises an alkylatable aromatic hydrocarbon.

17. The process of claim 3 further characterized in that said hydrocarbon starting material comprises essentially olefinic hydrocarbons.

18. The process of claim 4 further characterized in that it is carried out under a pressure of from about 1 to about 100 atmospheres.

19. A process for producing organic compounds of branched carbon structure which comprises contacting a reactive organic compound under conversion conditions with a catalyst comprising the reaction product formed by interacting a phosphoric acid and aluminum chloride and liberating hydrogen chloride in an amount not in excess of 2 mols for each mol of aluminum chloride present, whereby said reaction product contains at least one chlorine atom per mol.

20. A process for producing hydrocarbons of

5 branched carbon structure which comprises contacting a hydrocarbon material under reaction conditions with a catalyst comprising the reaction product formed by interacting a phosphoric acid and aluminum chloride and liberating hydrogen chloride in an amount not in excess of 2 mols for each mol of aluminum chloride present, whereby said reaction product contains at least one chlorine atom per mol.

10 21. A process for producing substantially saturated hydrocarbons of more-highly branched structure than that of a hydrocarbon starting material which comprises reacting said hydrocarbon material at a temperature of from about -20° to about 150° C. in the presence of a catalyst comprising the reaction product formed by interacting a phosphoric acid and aluminum chloride and liberating hydrogen chloride in an amount not in excess of 2 mols for each mol of aluminum chloride present, whereby said reaction product contains at least one chlorine atom per mol.

15 22. A process for producing substantially saturated hydrocarbons of more-highly branched structure than that of a hydrocarbon starting material which comprises reacting said hydrocarbon material at a temperature of from about -20° to about 150° C. in the presence of hydrogen chloride and of a catalyst comprising the reaction product formed by interacting a phosphoric acid and aluminum chloride and liberating hydrogen chloride in an amount not in excess of 2 mols for each mol of aluminum chloride present, whereby said reaction product contains at least one chlorine atom per mol.

20 23. A process for producing substantially saturated hydrocarbons of more-highly branched structure than that of a hydrocarbon starting material which comprises reacting said hydrocarbon material at a temperature of from about -20° to about 150° C. in the presence of hydrogen and a catalyst comprising the reaction product formed by interacting a phosphoric acid and aluminum chloride and liberating hydrogen chloride in amount not in excess of 2 mols for each mol of aluminum chloride present, whereby said reaction product contains at least one chlorine atom per mol.

VLADIMIR N. IPATIEFF.  
LOUIS SCHMERLING.